

Aug. 7, 1951

T. THOMSON ET AL

2,563,491

BLASTING ASSEMBLY

Filed July 11, 1947

FIG. 1.



FIG. 2.



Inventors:

THOMAS THOMSON and

KENNETH CATHRO REID

By

*Herb A. Wilson*  
Attorney

## UNITED STATES PATENT OFFICE

2,563,491

## BLASTING ASSEMBLY

Thomas Thomson, Kilmarnock, Ayrshire, and Kenneth Cathro Reid, Dundee, Scotland, assignors to Imperial Chemical Industries Limited, a corporation of Great Britain

Application July 11, 1947, Serial No. 760,308  
In Great Britain July 26, 1946

6 Claims. (Cl. 102—25)

1

The present invention relates to "Hydrox" blasting assemblies.

Within recent years the method of blasting with "Hydrox" has found application in the winning of coal from fiery and dusty mines on account of the exceptional safety characteristics as regards ignition of fire damp and coal dust-air mixtures and the comparatively gentle heaving action, which favours the production of lump coal, that result from the method. In the "Hydrox" blasting method there is used as the gas producing charge a quantity of "Hydrox powder" confined in a pressure resisting container having a closure adapted to yield at a predetermined and considerable pressure sufficient to produce a blasting effect when the gaseous and other products of reaction emerge into the bore hole. "Hydrox powder" is a mixture in granular form consisting essentially of a mixture of ammonium chloride and sodium nitrite stabilised by the inclusion of a small percentage of a faintly alkaline material. U. S. Patent No. 2,038,772 discloses a charge of sodium nitrite and ammonium chloride and U. S. Patent No. 2,190,460 discloses mixtures of sodium nitrite and ammonium chloride stabilized with magnesium oxide as the "Hydrox powder" set forth in this application.

The "Hydrox" blasting device normally includes a ported discharge head separated from the pressure resisting container by means of a steel disc adapted to yield at a predetermined pressure, so that when the pressure generated in this container by the "Hydrox powder" becomes sufficiently high the partly gaseous contents of the container rush into the discharge head, through the ports of which they stream into the bore hole, thus producing the blasting effect. The "Hydrox" blasting device normally includes also a firing head through which an electrically actuated local heating means embedded in the "Hydrox powder" and adapted to initiate its decomposition is connected with a source of current external to the device.

The possibility of "Hydrox" blasting depends on the fact that under atmospheric pressure conditions the "Hydrox powder" is capable of propagating through itself in a self-sustained fashion an exothermic reaction leading to the formation of nitrogen, steam and sodium chloride, when even a small portion of the mass of the granular mixture is heated to a suitable temperature. In the "Hydrox" blasting assembly the local heating means provided usually takes the form of an electric black powder fuse, which may conveniently contain up to 60 grains of black powder. Under the rising pressure conditions encountered in the pressure resisting container of the "Hydrox" blasting device, the decomposition of the "Hydrox powder" is greatly

accelerated, and the time between the completion of the electric circuit and the occurrence of the blast, which is mainly the time required for the decomposition of the "Hydrox powder" to complete itself after it has been initiated by the electric powder fuse, is usually only a fraction of a second; but even by increasing the charge in the electric black powder fuse it has not hitherto been practicable to reduce this time interval below about one fifth of a second.

In blasting operations it is often desirable to arrange that a plurality of blasts shall occur at the same instant, but the variations that are liable to occur in the aforesaid time intervals have hitherto been too great to enable simultaneous blasting effects to be obtained from a plurality of "Hydrox" blasting assemblies connected together in a single electric circuit.

The object of the present invention is to enable "Hydrox" blasting to be carried out with simultaneous occurrence of a plurality of shots.

We have now found that the time interval between the completion of the electric circuit and the venting of the products of decomposition of the "Hydrox powder" can be reduced to a period short enough to enable simultaneous blasting effects to be obtained from a plurality of "Hydrox" blasting devices electrically connected together for simultaneous shot firing when the electric black powder fuse is provided with a sheathing consisting of or comprising a perchlorate, particularly ammonium perchlorate.

In a "Hydrox" blasting device, therefore, according to the present invention the electric black powder fuse is provided with a sheathing consisting of or comprising a perchlorate particularly ammonium perchlorate.

It is assumed that in the presence of sufficient perchlorate the black powder fuse burns more vigorously and thus brings about the quicker ignition of the "Hydrox" powder. It is also assumed that during the burning of said fuse a substantial amount of hot perchlorate particles is projected into the surrounding granules of "Hydrox powder."

The invention also comprises a plurality of like "Hydrox" blasting devices electrically connected for simultaneous shot firing, said "Hydrox" blasting devices having each in addition to an electric powder fuse and a charge of "Hydrox powder" a charge consisting of or comprising a perchlorate, particularly ammonium perchlorate sheathing said electric powder fuse.

When the electric powder fuse is actuated, the hot products of the explosion of the black powder and the combustion of its paper container which include carbon monoxide and other oxidisable gases, undergo further oxidation with evolution of heat as they come into contact with the surrounding ammonium perchlorate, so that

the temperature of the gases is raised. The temperature of the unconsumed ammonium perchlorate being scattered by the explosion of the electric powder fuse is also raised sufficiently to cause it to undergo an exothermic decomposition into hot gaseous products. Moreover, the actively decomposing particles of ammonium perchlorate projected into contact with the "Hydrox powder" oxidise a portion of the sodium nitrited contained in these, again with the evolution of heat, and consequently an increase in the temperature of the gases already formed and an increase in the rate of decomposition of the ammonium perchlorate. The quantity of heat evolved in the form of hot gases is thus cumulatively increased, and the whole of the ammonium perchlorate is converted into hot gaseous products. Thus apart from the direct heating effects on "Hydrox powder" particles struck by the non-gaseous materials, the distributed heating effects on the particles of "Hydrox powder" permeated by hot gases far exceed what could be obtained by the use of the electric fuse alone before the cumulative effect of the normal decomposition of the "Hydrox powder" becomes effective, and the delay intervals can thereby be reduced to about 50 milliseconds or less.

It is desirable that the electric powder fuse, should contain not less than about the usual 60 grains of black powder for a 460 gram charge of "Hydrox powder" and the amount of ammonium perchlorate should be more than the quantity theoretically sufficient to oxidise the gases from the black powder and its paper container to carbon dioxide, water and sulphur dioxide, but not so great as to prevent its being scattered in an actively decomposing condition. About 20 grams is a suitable charge under these conditions. The "Hydrox powder" is preferably in a granulated condition. Under these conditions the time interval between completion of the circuit and the venting of the gases is about 30 milliseconds.

The invention is further illustrated in the diagrammatic drawings accompanying the specification whereof Figure 1 is a longitudinal section of a "Hydrox" blasting device embodying the invention and Figure 2 is a detailed diagrammatic drawing showing how a heater unit comprising an electric powder fuse is ensheathed in a charge of ammonium perchlorate.

In Figure 1, 1 is the pressure resisting container portion, 2 is the firing head, 3 is the discharge head and 4 is the bursting disc of a "Hydrox" blasting tube. 5 are the insulated leads from the firing head and 6 seen in greater detail in Figure 2 is the heater unit. 7 is a charge of "Hydrox powder No. 2."

In Figure 2, 5 are the insulated leads, 6 is a paper tube, 9 is a cork plug and 8 and 17 plugs of a polychloro-naphthalene wax. 10 is a paper disc and 11 is a charge of ammonium perchlorate. 12 is a paper tube, 13 and 14 are plugs of polychloro-naphthalene wax, 15 is a low tension electric fusehead. 16 is a charge of black powder. The items 12 to 16 constitute a 60 grain electric powder fuse, and the charge of ammonium perchlorate 11 amounts to 20 grams. The charge 7 of "Hydrox powder No. 2" in Figure 1 amounts to 460 grams.

We claim:

1. A blasting device of the kind comprising a pressure resisting steel contained having a closure adapted to yield at a predetermined and

4  
a considerable internal gas pressure and containing a charge in granular form consisting essentially of a mixture of sodium nitrite and ammonium chloride stabilized by the inclusion of a small percentage of a faintly alkaline material and electrically actuated local heating means wherein the local heating means comprises an electric black powder fuse enclosed in a sheathing consisting substantially of ammonium perchlorate.

5  
2. A blasting device as set forth in claim 1 having a weight of ammonium perchlorate sheathing in excess to that quantity theoretically sufficient to completely oxidize the combustion products resulting from the ignition of the black powder and yet a quantity not so great as to prevent it being scattered in an actively decomposing condition.

10  
3. A blasting device as set forth in claim 1 wherein approximately 60 grains of black powder and approximately 20 grams of ammonium perchlorate are present for each 460 gram charge of the blasting powder employed.

15  
20  
4. A plurality of blasting devices as set forth in claim 1 electrically connected for simultaneous firing.

25  
30  
35  
5  
An electric black powder fuse having a sheathing consisting substantially of ammonium perchlorate for use in a blasting device of the kind comprising a pressure resisting steel container having a closure adapted to yield at a predetermined and a considerable internal gas pressure and containing a charge in granular form consisting essentially of a mixture of sodium nitrite and ammonium chloride stabilized by the inclusion of a small percentage of faintly alkaline material and an electrically actuated heating means.

40  
6. An electric fuse for use in a blasting device of the kind comprising a pressure resisting steel container having a closure adapted to yield at a predetermined and a considerable internal gas pressure and containing a charge in granular form consisting essentially of a mixture of sodium nitrite and ammonium chloride stabilized by the inclusion of a small percentage of a alkaline material, said fuse comprising a core of black powder surrounded by a tubular casing, an electrical fuse head imbedded in the core, an ammonium perchlorate sheathing about said casing, and a second tubular casing enclosing said sheathing, each end of the said casings being sealed.

THOMAS THOMSON.  
KENNETH CATHRO REID.

#### REFERENCES CITED

The following references are of record in the file of this patent:

#### UNITED STATES PATENTS

| Number    | Name         | Date          |
|-----------|--------------|---------------|
| 1,950,038 | Scott        | Mar. 6, 1934  |
| 2,038,772 | Taylor       | Apr. 28, 1936 |
| 2,075,969 | White et al. | Apr. 6, 1937  |
| 2,190,460 | Taylor       | Feb. 13, 1940 |

#### FOREIGN PATENTS

| Number           | Country       | Date                        |
|------------------|---------------|-----------------------------|
| 2,926<br>of 1899 | Great Britain | Feb. 9, 1900                |
| 15,512           | France        | July 25, 1912<br>(Addition) |
| 424,785          | Great Britain | Feb. 28, 1935               |
| 544,252          | Great Britain | Apr. 3, 1942                |